

March 7, 1967

R. J. FOREMAN ET AL  
THERMIONIC EMISSIVE CATHODE WITH END  
STRUCTURE FOR EMISSIVE SUPPRESSION  
Filed Nov. 23, 1962

3,308,329



INVENTOR'S

Robert J. Foreman  
Joseph A. Smith

BY

*Robert E. Strauss*  
ATTORNEY

## 1

3,308,329

**THERMIONIC EMISSIVE CATHODE WITH END STRUCTURE FOR EMISSIVE SUPPRESSION**  
Robert J. Foreman and Joseph A. Smith, Williamsport, Pa., assignors, by mesne assignments, to Litton Industries, Inc., Beverly Hills, Calif., a corporation of DelawareFiled Nov. 23, 1962, Ser. No. 239,453  
2 Claims. (Cl. 313—107)

This invention relates to barium-containing cathode structures used in evacuated thermionic electron emissive devices, and more particularly to a cathode structure for use in a microwave device such as a magnetron wherein discrete areas of the cathode supporting structure are covered with a layer of alloyed material having both emission suppression and gettering properties.

In evacuated electron emissive devices it is important to have the electron emission confined to the intended cathode area in order that proper functioning of the devices can be consistently maintained. It is a common practice in certain of these devices such as magnetrons to incorporate annular flanges transversely positioned one on either end of the cathode emitting surface to serve as end shields to block or prevent longitudinal electron escape from the cathode-anode interaction space into the end spaces flanking the anode. The internal geometry of the tube structure is such that the peripheral edge of each end shield is proximal to a magnet pole piece.

During both the standby and operating states of tube operation there is migration of electron emitting materials from the cathode emitting surface onto the adjacent end shields thereby creating areas of spurious emission. Upon alteration of the operational status of the tube such as when switching from standby to full operation or the changing of pulse lengths or duty cycle, the areas of spurious emission on the end shields create periods of undesirable operational instability.

Since there is a closeness of end shield and pole piece spacing and vastly different operational electrical potentials existent therebetween, spurious emission in that region acting in conjunction with the magnetic and electric fields of the device constitutes an electron beam extending between the end shield and the neighboring pole piece. This detrimental condition, known in the art as high energy hollow beams, is capable of inducing arcing and causing severe erosion of the steel pole piece with the resultant production of sputtered metal and deleterious gases. These in turn aggravate an erratic arcing situation and bring about a reduction in cavity Q which further lowers the operational efficiency and reliability of the tube.

To overcome spurious emission and its consequences, a number of materials and coatings for the end shields and contiguous structures have been tried, but the disadvantages very often outweighed the intended advantages. One of these remedial measures was to employ end shields fabricated from a pure zirconium metal which exhibits well-known properties of emission suppression and gettering. Pure zirconium was found to be unsatisfactory since it undergoes a transformation of crystalline structure (phase change) at a temperature lower than the normal tube processing and operating temperatures. Consequently, end shields formed of zirconium displayed severe structural distortion. When unalloyed zirconium was applied alone as coating, there was a noticeable lack of satisfactory adherence. The shedding of the loose zirconium particles on handling made unalloyed zirconium both undesirable and unacceptable for this particular usage. Moreover, the porous sintered layer of zirconium exhibited inferior emission suppression capability.

## 2

Accordingly, it is an object of this invention to reduce the aforementioned disadvantages by providing a cathode structure that has defined areas covered with an alloy material which advantageously presents a smooth non-porous surface which evidences no noticeable damage when subjected to elevated temperatures.

It is a further object to provide a layer of alloy material that has adequate coverage depth and adherence capabilities and which can be handled readily without encountering surface damage.

It is an additional object to provide a layer of alloy material that exhibits both emission suppression and gettering properties.

The foregoing objects are achieved in one aspect of the invention by vacuum firing a layer of zirconium-nickel mixture to discrete areas of the end shields and the cathode supporting structure. The alloy material so formed demonstrates excellent oxide reduction and gettering properties, exhibits good coverage of the areas concerned, surface alloys well with the refractory metal base material, and undergoes no serious degree of distortion at tube processing and operating temperatures.

For a better understanding of the present invention, together with other and further objects, advantages, and capabilities thereof, reference is made to the following disclosure and appended claims in connection with the accompanying drawing in which an enlarged plan view shows a portion of a cathode structure and related tube parts.

Referring to the figure, cathode assembly structure 11 consists of a hollow cylindrical base or spindle member 13 fabricated from a refractory metal such as molybdenum which is capable of withstanding high operational temperatures. This cathode assembly structure 11 is designed for orientation in spaced relationship with the anode structure 15 and steel magnet pole pieces 17 and 17' which have therein longitudinal bores 19 and 19' to facilitate the mounting of assembly structure 11. A sleeve-type dispenser cathode 21 composed of a tungsten matrix impregnated with an electron emitting composition such as barium aluminate is positioned on spindle member 13 in spaced relationship with anode structure 15. An insulated tungsten heater 23 of conventional design is suitably mounted within cathode assembly structure 11 in heat relationship with cathode 21 to facilitate thermionic electron emission therefrom. An annular flange or end shield 25, likewise of molybdenum or tungsten, is integrally formed on spindle member 13 to provide a barrier to electrons attempting to leave the interaction space 48 and enter the adjacent end space 50. Any electrons outside the interaction space constitute waste current which reduces tube efficiency.

A similar protective construction is embodied in another annular flange or end shield 27, similar to flange 25, but integrally attached to a molybdenum sleeve 29. This end shield sleeve 29 has an internal diameter slightly larger than the external terminal diameter of spindle 13 enabling a slidable fit thereon to abut the cathode 21, whereupon sleeve 29 is fastened to spindle member 13 as by welding, brazing, or a similar means of securement. This second annular flange or end shield 27 functions similarly to previously described shield 25 in that it acts as a barrier to electrons attempting to enter end space 52.

A coating of zirconium-nickel mixture is discretely applied to end shield sleeve 29 and vacuum fired prior to the mounting of sleeve 29 on spindle 13. While this process will be fully described later, it is appropriate to mention that during vacuum firing, when temperatures between 1500°-1700° C. are encountered, the Zr-Ni mixture melts, wets, and alloys with the molybdenum sleeve and forms thereon a smooth, nonporous surface

layer of zirconium alloy 31. During the firing process excess nickel evaporates thereby raising the melting point of the resultant zirconium alloy layer to temperatures well above 1200° C.; the highest temperature to which the cathode assembly structure will be subjected to either during tube processing or subsequent operation.

In considering the completed cathode assembly structure 11, the layer of zirconium alloy 31 begins at a concentrical boundary 35 on annular flange 27 which is substantially midway on the surface of flange 27 facing the cathode 21. The alloy layer 31 which progresses over the periphery 28 of flange 27 covers the remainder of the flange and continues along the end shield sleeve 29 to a boundary 37 near the end of the sleeve. From concentrical boundary 35 to cathode 21 there is a bare surface sleeve area 39 that is devoid of zirconium alloy. This bare surface provides a barrier intended to prevent migration of zirconium to the cathode emitting surface.

There is a like layer of zirconium alloy 40 integrally attached to a defined surface area of spindle member 13 beginning at a concentrical boundary 41 on annular flange 25 which is likewise substantially midway on the surface of flange 25 facing cathode 21. This alloy layer progresses over the periphery 26 of flange 25 and covers the remainder of the flange and continues along spindle 13 to a terminal boundary 43 thereon which is substantially within bore 19 of magnet pole piece 17. It will also be noted that from concentrical boundary 41 to cathode 21 there is a bare surface spindle area 45 that is devoid of zirconium alloy similar to the bare surface sleeve area 39 mentioned above.

The significance of the zirconium-nickel alloy material may be more fully explained in the following manner. By selection, peripheries 26 and 28 of molybdenum end shield flanges 25 and 27 respectively are spaced adjacent surfaces 18 and 18' of steel magnet pole pieces 17 and 17'. When a tube is under operating conditions, a full pulse voltage will exist between pole piece surface 18 and flange periphery 26; and the same is true between pole piece surface 18' and flange periphery 28. In addition, there is also present in this region a permanent magnetic field of considerable magnitude which is parallel to the electric field. As previously mentioned, if stray electrons are present in the end spaces, these two fields constitute contributory conditions for the formation of a high energy electron beam, thus making that region of the tube particularly vulnerable to detrimental arcing. During cathode activation at approximately 1170° C. and in subsequent standby and operational conditions wherein the cathode is at a temperature of 900° C. to 990° C., there is migration of barium, barium oxide, and other cathode materials from the surface of the cathode to adjacent surfaces such as those of the neighboring end shield structure. Defined end shield and spindle areas adjacent to the cathode 21 of cathode assembly structure 11 are adequately covered with a layer of alloy material 31 and 40 that has emission suppression and gettering properties.

As previously stated, sintering on pure zirconium powder is not satisfactory since the adherence is poor and the surface emission suppression capability is inferior. Moreover, end shields of pure solid zirconium undergo a transformation of crystalline structure at a temperature of 862° C. which causes severe surface deterioration. It has been found that by alloying another metal such as nickel with zirconium, no serious surface destruction is observed.

In the preferred embodiment, zirconium, because of its emission suppression and gettering properties, is desired as the predominant metal in the alloy. When combined with nickel, the resulting alloy exhibits improved qualities of surface coverage and bonding. It has been found that when the Zr-Ni mixture is applied and alloyed to the molybdenum base members 13 and 29, the surface of the molybdenum diffuses into the zirconium and nickel

alloy to provide an interface ternary Zr-Ni-Mo alloy. While information as to the exact conditions required to form the Zr-Ni-Mo interface combination are not fully known, it is known that the desired alloying results can be accomplished within the temperature range of 1500° C. to 1700° C., depending upon the Zr-Ni mixture employed. By increasing the weight percentage of nickel in the Zr-Ni mixture towards the eutectic composition (17%), the temperatures required for alloy formation can be reduced to facilitate rapid alloying for various designs of cathode spindle member 13 within temperatures safe for the structures involved.

To achieve the desired Zr-Ni-Mo alloying, it has been found that the proportion of zirconium in the Zr-Ni mixture may be varied within the range of 83 percent to 96 percent by weight. This weight percentage range for the Zr-Ni mixture represents the proportions wherein the most advantageous temperature alloying results can be achieved. The terminal percentage values are not critical limits defining success or failure; they are representative values above and below which results of lesser desirability will be encountered. It is desired to have as high a zirconium content as possible; but as the amount of zirconium is increased, the required alloying temperature also rises and inferior surface coverage is evidenced. Experience has shown that proportional variations within the aforementioned range have yielded desired results. The eutectic temperature for the Zr-Ni composition by weight of 83 percent zirconium and 17 percent nickel is 961° C. At the upper end of the preferred compositional range, if the zirconium content is increased above 96 percent, the gradient of the alloying temperature rises to a value above 1600° C. which approaches the critical temperature for embrittlement of the molybdenum base members which in some applications may be undesirable.

The zirconium content of the Zr-Ni-Mo alloy exhibits the inherent reducing properties of zirconium. The barium and barium oxide migrating from the cathode 21 comes in contact with the Zr-Ni-Mo material. The barium oxide rapidly undergoes a reduction reaction wherein zirconium oxide is formed and barium is released and evaporated from the Zr-Ni-Mo surface. The zirconium oxide thus formed is a very stable compound at the highest temperatures encountered during tube activation and operation. Thus the elimination of the spurious electron emission from migratory emitting deposits prevents the formation of the high energy hollow beam previously described, and tube operational stability and efficiency are greatly improved.

Zirconium is also prominent as an efficient high temperature gettering element and, like all chemical gettering materials, tends to have diminishing ability due to the formation of oxides, nitrides, etc. on its surface. As a result, after tube activation and exhaust processing temperatures of 1150° C. to 1170° C., its surface gettering ability is greatly reduced. However, since there is an abundance of subsurface alloyed zirconium on the end shield flanges 25 and 27 adjacent magnet pole surfaces 18 and 18', where arcing in magnetrons generally occurs, the occurrence of an arc disrupts the surface compounds on the alloy material 31 and 40 and exposes a new surface of active zirconium underneath. Arcing vaporizes a small amount of metallic zirconium which combines not only with gases released during the arc but also with the gas which was responsible for initiating the arc originally. Thus a regenerative gettering or pumping action is constantly available within the tube as the need may manifest itself during continued operation. This reserve gettering ability has the resultant benefit of maintaining desirable gas levels within the tube, whereby life expectancy of high power magnetrons is appreciably extended.

An added benefit of the alloy layer is the surface characteristic thereof which, being somewhat darkened, has

improved heat radiating qualities. This factor is advantageous in high power high frequency magnetron devices to aid in the dissipation of heat derived from back bombardment of the cathode.

The process for applying and alloying the Zr-Ni mixture to the molybdenum end shield sleeve 29 and the molybdenum spindle member 13 is accomplished on each respective part before the assembly of the combination.

The procedure begins with the constitution of the Zr-Ni material. Both the zirconium and nickel powders comprising the mixture have particle sizes ranging from two to four microns. They are mixed dry only in small batches of four or five grams since zirconium is highly reactive to oxygen and therefore susceptible to spontaneous combustion. As a safety precaution, wet mixing is recommended if larger size batches are considered. As a safety expedient, zirconium hydride powder may be employed in place of the pure zirconium powder in the mixture.

The mixture of zirconium and nickel powders are suspended in a volatile organic binder such as nitrocellulose lacquer. A solvent such as for example amyl acetate is added to thin the mixture to a consistency proper for application to achieve desired coverage and adherence. The volatile nature of the amyl acetate makes for variable liquid consistency; but it has been found that a suspension viscosity of approximately 100 cps. is quite satisfactory for facile application of the mixture to the base members. If the suspension is too viscous, peeling may result upon the application of heat during vacuum firing.

The method for applying the Zr-Ni mixture is not critical as long as the desired area of the base member is adequately covered with a layer of Zr-Ni material of consistent thickness. Experimentation has shown that a finished alloy thickness of two mils is considered a minimum requirement to insure adequate coverage. The desired thickness for satisfactory coverage may be achieved by a build-up of two or more individually processed layers. There is no definite maximum thickness since complete surface coverage fulfills the essential requirements. Internal spacings and design dimensions must be considered accordingly. The application technique usually employed involves a means for rotating the base member parts while the Zr-Ni suspension is applied by fine jet air spray or brush. The rotation for application of the Zr-Ni metal to the respective individual parts is facilitated by utilizing the chuck of a lathe for grasping end portion 47 of shield sleeve 29 and shank portion 49 of spindle member 13.

In the alloying process, the shield sleeve 29 is temporarily placed on the terminal end of the spindle member 13 and the two coated members are temperature processed simultaneously. This alloying is executed in a vacuum furnace at a pressure not to exceed  $5 \times 10^{-5}$  mm. Hg.

The actual alloying is rapidly accomplished during a ten second interval at a temperature within the range of 1500° C. to 1700° C. The exact temperature is dependent upon the proportional composition of the Zr-Ni mixture that is to be alloyed with the molybdenum surfaces to which the suspension has been applied. Since recrystallization of the molybdenum follows a time-temperature relationship, it is desirable to accomplish rapid alloying of the Zr-Ni layer to the molybdenum surface before the whole of the molybdenum structure can be subjected to the time-temperature criticality for embrittlement.

As heretofore mentioned, the weight percentages of zirconium and nickel in the alloy can be varied within the aforementioned range to facilitate alloying with respect to the size and mass of the cathode assembly structure concerned without materially lessening the benefits of the zirconium content. This permits a variation of the processing temperatures with the time factor remaining constant.

During the high temperature vacuum firing, of short time duration, there is a chemical breakdown of the Zr-Ni suspension whereupon the amyl acetate and nitrocellulose binder are volatilized. A portion of the nickel content is vaporized from the surface of the alloy. While the exact nickel content of the final alloyed layer is not definitely known, it is evidenced from processing that the higher the nickel content of the alloy the greater the amount of nickel vaporization. Due to the short duration of high temperature processing, it is believed that most of the vaporized nickel comes from the outer molecular layers of the alloy surface.

While nickel has been described as the preferred metal to be added to the zirconium, several other finely divided or powdered transition metals can be similarly used in proper proportional combinations with zirconium under suitable temperature conditions. For this application the material to be successfully alloyed with zirconium should be a metal having a favorable vapor pressure at the operating temperature of the cathode and one of which a minor quantity will effect a resultant reduction in the melting point of zirconium to within the range of 1500° C. to 1700° C. In addition to nickel, suitable transition metals would include cobalt, vanadium, titanium, chromium, manganese, molybdenum, and tungsten. Some examples of zirconium alloy weight combinations are:

| Percentage-Weight Combination of Powder Mixture | Alloy Mixture              | Eutectic Temperature, ° C. |
|-------------------------------------------------|----------------------------|----------------------------|
| 50:50                                           | Zirconium-titanium -----   | 1,610                      |
| 70:30                                           | Zirconium-vanadium -----   | 1,230                      |
| 82:18                                           | Zirconium-chromium -----   | 1,300                      |
| 77.5:22.5                                       | Zirconium-manganese -----  | 1,135                      |
| 69:31                                           | Zirconium-molybdenum ----- | 1,520                      |
| 82:18                                           | Zirconium-tungsten -----   | 1,650                      |

There has thus been described a cathode structure adapted for use in a magnetron structure whereon there has been provided a layer of alloy material having reduction and gettering properties. This material is integrally alloyed with specific areas associated with the cathode assembly structure and exhibits excellent adherence, adequate coverage, and evidences excellent emission suppression and gettering ability. This results in a vast improvement in stability of tube performance and lengthening of operational life. It has been found that leakage current and gas content within the tube have materially decreased during operational usage thereby achieving substantial gains in overall tube performance and efficiency. Tubes which have been subjected to a reaging process, necessitated by operational abuse or arcing, have successfully completed a considerable degree of extended life.

While not shown, the essentials of this invention are equally adaptable to usage in traveling wave tubes, backward wave oscillators, klystrons, and similar devices wherein it is desirable to have discrete areas of high temperature operating electrodes exhibit emission suppression and gettering properties to enhance operational efficiency. The desired alloy mixture is applied as a coating to specific regions of the refractory metal electrode structures and vacuum fired for alloying as previously described.

While there has been shown and described what is at present considered the preferred embodiments of the invention, it will be obvious to those skilled in the art that various changes and modifications may be made therein without departing from the scope of the invention as defined by the appended claims.

What is claimed is:

1. A cathode assembly structure adapted for use in an evacuated high temperature thermionic emissive

- device having an anode and oppositely spaced pole pieces with axially aligned longitudinal bores comprising:
- a tubular spindle axially positioned and spaced to extend through said anode and into the longitudinal bores of said pole pieces, 5
  - a thermionic cathode, employing barium compounds capable of providing electron emission, mounted on said spindle in spaced relationship with said anode, transversely outstanding annular flanges functioning as emission end shields mounted on said spindle and spaced from each end of said cathode and adjacent the openings of said longitudinal bores, and 10
  - a continuous layer of a zirconium-nickel alloy having emission suppression and gettering properties integral with and extending along at least a portion of 15 said flanges and said spindle to a position substantially within said bores.
2. A cathode assembly structure adapted for use in an evacuated high temperature thermionic electron emissive device having an anode and oppositely spaced pole pieces with axially aligned longitudinal bores comprising:
- a tubular spindle axially positioned and spaced to extend through said anode and into the longitudinal bores of said pole pieces,

a thermionic cathode, employing barium compounds capable of providing electron emission, mounted on said spindle in spaced relationship with said anode, transversely outstanding annular flanges functioning as emission end shields mounted on said spindle and spaced from each end of said cathode and adjacent the openings of said longitudinal bores, and a continuous layer of zirconium-nickel alloy of which zirconium comprises more than 83 percent by weight, bonded to at least a portion of said flanges and extending along said spindle providing emission suppression and gettering properties thereon.

## References Cited by the Examiner

## UNITED STATES PATENTS

|           |         |                 |       |           |
|-----------|---------|-----------------|-------|-----------|
| 2,491,284 | 12/1949 | Sears           | ----- | 313—178 X |
| 2,647,216 | 7/1953  | Brown           | ----- | 313—157   |
| 2,957,100 | 10/1960 | Espersen et al. | ----- | 313—346   |

20 JAMES W. LAWRENCE, *Primary Examiner.*

GEORGE N. WESTBY, *Examiner.*

P. C. DEMEO, *Assistant Examiner.*